

# UNITED STATES PATENT OFFICE.

HANS WALther, OF LEVERKUSEN, NEAR COLOGNE, GERMANY, ASSIGNOR TO  
SYNTHETIC PATENTS CO., INC., OF NEW YORK, N. Y., A CORPORATION OF  
NEW YORK.

## COTTON MATERIAL WITH WHITE-EFFECT THREADS AND PROCESS OF MAKING IT.

1,270,348.

Specification of Letters Patent. Patented June 25, 1918.

No Drawing.

Application filed November 5, 1914. Serial No. 870,492.

*To all whom it may concern:*

Be it known that I, HANS WALther, doctor of philosophy, chemist, citizen of the German Empire, residing at Leverkusen, 5 near Cologne, Germany, have invented new and useful Improvements in Cotton Materials with White-Effect Threads and Processes of Making Them, of which the following is a specification.

10 I have found that in dyeing cotton piece goods with sulfurized dyestuffs, silk color effect threads can be protected from being dyed by treating the goods before dyeing with tanning substances which may preferably be fixed on the fiber by means of tar- 15 tar emetic or formaldehyde, etc. White effects are thus obtained, especially when using mercerized cotton.

Example 1: Textile goods consisting of 20 cotton and silk are mercerized under tension by means of a caustic soda lye of 30° Bé., rinsed, neutralized, laid into a bath during 12 hours which contains 5 grams of tannin per liter of dye liquor subsequently used and then into a second bath containing 25 2 grams of tartar emetic per liter of dye liquor, the dye liquor subsequently used. Subsequently the fabric thus mercerized and 30 mordanted with tannin is dyed in a bath of the following composition:

25 per cent. of Katigen black BFC extra. 25 per cent. of crystallized sodium sulfid. 3 grams of sodium carbonate. } per liter 35 40 grams of common salt. } of dye 50 30 grams of glue. } liquor.

The color effect threads contained in the goods are pure white while the cotton appears deep black.

40 Example 2: Cotton goods containing silk

color effect threads and mercerized and mordanted with tannin as above described, are treated during half an hour at 60° C. with a 2 per cent. formaldehyde and are then dyed at 30-40° C. in a bath of the following 45 composition:

30 per cent. of Katigen brilliant green 3G. 30 per cent. of crystallized sodium sulfid. 3 grams of sodium carbonate. } per liter 50 40 grams of common salt. } of dye 50 30 grams of glue. } liquor.

The silk threads are white while the cotton appears green.

In the same way mixed goods can be 55 treated.

I claim:

1. Process of resisting the silk in mixed goods in the operation of dyeing them with sulfurized dyestuffs, consisting in treating 60 the goods to be dyed with tanning substances, substantially as described.

2. The process of producing silk white effect goods dyed with sulfur colors which comprises subjecting mixed cotton and silk 65 goods to tannin and subsequently dyeing the goods with sulfur colors in a bath containing a metal sulfid.

3. A textile material having white effects, and comprising a mixture of cotton and silk, 70 the latter being mordanted with tannin, the cotton only of said mixture being dyed with sulfur colors, substantially as described.

In testimony whereof I have hereunto set my hand in the presence of two subscribing 75 witnesses.

HANS WALther.

Witnesses:

LEE LEHOENTHAL,  
L. H. MARSHALL.